

Aug. 19, 1958

J. J. CHECHAK ET AL

2,848,329

SUPERSENSITIZATION WITH BIS-HETEROCYCLIC BASES

Filed May 14, 1956

**Fig.1**



A=3,3'-DIETHYLTHIADICARBOCYANINE IODIDE  
B=3,3'-DIETHYLTHIADICARBOCYANINE IODIDE WITH 1,4-[2-(5-PHENYLOXAZOLYL)] BENZENE

**Fig.2**



C=3,3'-DIETHYLTHIADICARBOCYANINE IODIDE  
D=3,3'-DIETHYLTHIADICARBOCYANINE IODIDE WITH 1,2-BIS(2-BENZOTHIAZOLYL) ETHYLENE

**Fig.3**



E=3,3'-DIETHYLOXADICARBOCYANINE IODIDE  
F=3,3'-DIETHYLOXADICARBOCYANINE IODIDE WITH 1,4-BIS[2-(5-PHENYLOXAZOLYL)] BENZENE

**Jonas J. Chechak  
Jean E. Jones**

INVENTORS

*Daniel J. Mayne*  
BY

*Lawrence H. Willis*

ATTORNEYS

2,848,329

## SUPERSENSITIZATION WITH BIS-HETEROCYCLIC BASES

Jonas John Chechak and Jean E. Jones, Rochester, N. Y., assignors to Eastman Kodak Company, Rochester, N. Y., a corporation of New Jersey

Application May 14, 1956, Serial No. 584,544

10 Claims. (Cl. 96—104)

This invention relates to photographic silver halide emulsions useful in color photography and photographic silver halide emulsions containing dicarbocyanine dyes, and as supersensitizers therefor, certain heterocyclic bases.

It is known in the art of making photographic emulsions that certain dyes of the cyanine class alter the sensitivity of photographic emulsions of the gelatin-silver-halide kind, when the dyes are incorporated in the emulsions. It is also known that the sensitization produced by a given dye varies somewhat with the type of emulsion in which the dye is incorporated. Furthermore, the sensitization of a given emulsion by a given dye may be altered by varying the conditions in the emulsion. For example, the sensitization may be increased by increasing the silver ion concentration or decreasing the hydrogen ion concentration (i. e., increasing the alkalinity) or both. Thus, sensitization can be increased by bathing plates, coated with a spectrally sensitized emulsion, in water or in aqueous solutions of ammonia. Such a process of altering the sensitivity of a sensitized emulsion by increasing the silver ion concentration and/or by decreasing the hydrogen ion concentration is commonly called "hypersensitization." Hypersensitized emulsions have generally poor keeping qualities.

We have now found another means of altering the sensitivity in emulsions containing dicarbocyanine dyes. Since the conditions in the emulsion, i. e., the hydrogen ion and/or the silver ion concentration undergo little or no change in our method, we shall designate our method as a kind of supersensitization.

It is, therefore, an object of our invention to provide photographic emulsions containing dicarbocyanine dyes and, as supersensitizers therefore, certain heterocyclic bases. Another object is to provide a process for preparing these supersensitized emulsions. Other objects will become apparent from a consideration of the following description and examples.

The dicarbocyanine dyes which are useful in practicing our invention include those represented by the following general formula:



wherein R and R<sub>1</sub> each represents an alkyl group (such as methyl, ethyl,  $\beta$ -hydroxyethyl, carboxymethyl,  $\beta$ -carboxethyl, carbomethoxymethyl, carbethoxymethyl, etc.), n represents a positive integer of from 1 to 2, X represents an acid radical, such as chloride, iodide, bromide, perchlorate, p-toluenesulfonate, benzenesulfonate, ethylsulfate, methylsulfate, etc., Z represents the non-metallic atoms necessary to complete a heterocyclic nucleus containing from 5 to 6 atoms in the heterocyclic ring, e. g., a heterocyclic nucleus of the benzothiazole series (e. g., benzothiazole, 4-chlorobenzothiazole, 5-chloro-

benzothiazole, 6-chlorobenzothiazole, 7-chlorobenzothiazole, 4-methylbenzothiazole, 5-methylbenzothiazole, 6-methylbenzothiazole, 5 - bromobenzothiazole, 6 - bromobenzothiazole, 4-phenylbenzothiazole, 5-phenylbenzothiazole, 4-methoxybenzothiazole, 5 - methoxybenzothiazole, 6 - methoxybenzothiazole, 6 - iodobenzothiazole, 5 - iodo-benzothiazole, 4-ethoxybenzothiazole, 5-ethoxybenzothiazole, 5,6-dimethylbenzothiazole, 5-hydroxybenzothiazole, 6-hydroxybenzothiazole, etc.), a heterocyclic nucleus of the naphthothiazole series (e. g.,  $\alpha$  - naphthothiazole,  $\beta$ -naphthothiazole, 7-methoxy- $\alpha$ -naphthothiazole, 8-methoxy -  $\alpha$  - naphthothiazole, 5 - methoxy- $\beta$ -naphthothiazole, 5-ethoxy- $\alpha$ -naphthothiazole, etc.), a heterocyclic nucleus of the benzoselenazole series (e. g., benzoselenazole, 5 - chlorobenzoselenazole, 6 - methoxybenzoselenazole, 5-methoxybenzoselenazole, etc.), a heterocyclic nucleus of the naphthoselenazole series (e. g.,  $\alpha$ -naphthoselenazole,  $\beta$ -naphthoselenazole, etc.), a heterocyclic nucleus of the benzoxazole series (e. g., benzoxazole, 5-hydroxybenzoxazole, 6-hydroxybenzoxazole, 5-chlorobenzoxazole, 5-methoxybenzoxazole, 6-methoxybenzoxazole, 5-phenylbenzoxazole, 5-bromobenzoxazole, etc.), a heterocyclic nucleus of the naphthoxazole series (e. g.,  $\alpha$ -naphthoxazole,  $\beta$ -naphthoxazole, etc.), a heterocyclic nucleus of the 2-quinoline series (e. g., 2-quinoline, 6-methyl-2-quinoline, 7-methyl-2-quinoline, 8-methyl-2-quinoline, 6-chloro-2-quinoline, 7-chloro-2-quinoline, 5 - ethoxy-2-quinoline, 6 - ethoxy-2-quinoline, 7-ethoxy-2-quinoline, 6-methoxy-2-quinoline, etc.), a heterocyclic nucleus of the 4-quinoline series (e. g., 4-quinoline, 6-methoxy-4-quinoline, 7-methyl - 4 - quinoline, 8-methyl-4-quinoline, etc.), a heterocyclic nucleus of the benzimidazole series (e. g., benzimidazole, 5-chlorobenzimidazole, 5,6-dichlorobenzimidazole, 1,7-trimethylenebenzimidazole, etc.), a heterocyclic nucleus of the 5,6 - benzoquinoline series (e. g., 5,6-benzo-2-quinoline, etc.), etc., and Z<sub>1</sub> represents the non-metallic atoms necessary to complete a heterocyclic nucleus selected from the group consisting of those of the quinoline series (e.g., such as those defined by Z above), those of the benzoxazole series (e. g., such as those defined by Z above), those of the naphthoxazole series (e. g., such as those defined by Z above), those of the benzoselenazole series (e. g., such as those defined by Z above), those of the naphthoselenazole series (e. g., such as those defined by Z above), those of the benzothiazole series (e. g., such as those defined by Z above), those of the naphthothiazole series (e. g., such as those defined by Z above), etc. Other carbocyanine dyes can also be employed in our invention.

The heterocyclic bases useful in practicing our invention comprise heterocyclic nitrogen bases containing from 1 to 2 nitrogen atoms and having a substituent attached thereto which contains at least four carbon atoms. Such heterocyclic bases comprise those advantageously represented by the following general formula:



wherein Z<sub>2</sub> represents the non-metallic atoms necessary to complete a heterocyclic nucleus containing from 1 to 2 nitrogen atoms in the heterocyclic ring (e. g., those of the thiazole series, those of the benzothiazole series, those of the naphthothiazole series, those of the oxazole series, those of the benzoxazole series, those of the naphthoxazole series, those of the selenazole series, those of the benzoselenazole series, those of the naphthoselenazole series, those of the benzimidazole series, those of the quinoline series, etc.), and R<sub>2</sub> represents an organic radical containing at least 4 carbon atoms, said radical hav-

ing a molecular weight of at least 71. Embraced by the above general Formula II are the bis-heterocycl compounds represented by the following general formula:

(III)



wherein  $Z_2$  has the values given above,  $d$  represents a positive integer of from 1 to 2, and  $D$  represents a divalent organic radical, such as dithiaalkylene (e. g.,  $\alpha,\omega$ -dithiaalkylene groups, such as  $\alpha,\omega$ -dithiapropane,  $\alpha,\omega$ -dithiabutylene,  $\alpha,\omega$ -dithiapentylene, etc., especially such groups containing from 1 to 5 carbon atoms), alkylene (e. g., methylene, ethylene, propylene, butylene, pentylene, hexylene, etc., especially such groups containing from 1 to 10 carbon atoms), arylene (e. g., phenylene, biphenylene, benzylene, bis(phenylene)methyl, etc., especially such groups containing from 6 to 13 carbon atoms), vinylene, thio, oxydimethylene, etc. Typical bis-heterocyclic compounds represented by Formula III include the following:

(1)



1,5-bis(2-benzothiazolylthio)pentane

(2)



1,2-bis(2-benzothiazolyl)ethane

(3)



1,3-bis(2-benzothiazolyl)propane

(4)



1,4-bis(2-benzothiazolyl)butane

(5)



1,5-bis(2-benzothiazolyl)pentane

(6)



Bis(2-benzothiazolylthio)methane

(7)



1,2-bis(2-benzothiazolylthio)ethane

(8)



Bis(2-benzothiazolyl)sulfide

(9)



Bis[4-(2-benzothiazolyl)phenyl]methane

(10)

5

1,4-bis(2- $\alpha$ -naphthothiazolyl)butane

10 (11)

Bis(2- $\alpha$ -naphthothiazolyl)methane

15 (12)



p,α-Bis(2-benzothiazolyl)toluene

20 (13)



Bis(2-benzothiazolylmethyl)ether

25 (14)

Bis(2- $\beta$ -naphthothiazolyl)methane

30 (15)



1,4-bis(2-benzimidazolyl)benzene

35 (16)



1,4-bis(5-phenyl-2-oxazolyl)benzene

40 (17)



Bis(2-benzothiazolyl)methane

45 (18)



1,2-bis(2-benzimidazolyl)ethylene

50 (19)



2-(2-benzothiazolyl)benzothiazole

55 (20)



1,5-bis(2-benzoxazolyl)pentane

5



Also embraced by Formula II above are heterocyclic bases selected from those represented by the following general formula:



wherein  $Z_2$  has the values given above and  $R_3$  represents an alkyl group (e. g., amyl, hexyl, octyl, decyl, dodecyl, etc., especially an alkyl group containing from 5 to 12 carbon atoms), an aryl group (e. g., phenyl, o-, m-, and p-tolyl, o-, m-, and p-anisyl, o-, m-, and p-aminophenyl, p-dimethylaminophenyl, p-diethylaminophenyl, etc., especially a mononuclear aromatic group of the benzene series), an aralkyl group (e. g., benzyl,  $\beta$ -phenylethyl, etc.), an aryloxyalkyl group (e. g., phenoxyethyl,  $\beta$ -phenoxyethyl, etc.), an acylamido group (e. g., butyramido toluamido, acetacetamido, valeramido, benzamido, etc., especially an acylamido group containing from 4 to 9 carbon atoms), alkylmercapto, arylmercapto, a substituted amino group (e. g., butylamino, anilino, tolyl-amino, etc.), and a substituted imino group. Bases embraced by Formula IV include the following:



2,848,329

6



70 As shown above, the heterocyclic nuclei represented by  $Z_2$  of Formula II above can have substituents thereon which do not interfere with the photographic emulsion. Such substituents can be alkyl groups, such as methyl, ethyl, etc., aryl groups, such as phenyl, tolyl, etc., halogen atoms, such as chlorine, bromine, etc., alkoxy

75

groups, such as methoxyl, ethoxyl, etc., hydroxyl, amino, etc.

According to our invention, we incorporate one or more of the dicarbocyanine dyes represented by Formula I above with one or more heterocyclic bases, such as those represented by Formulas II, III or IV above. Our invention is particularly directed to the ordinarily employed gelatino-silver-halide emulsions. However, our supersensitizing combinations can be employed in silver halide emulsions in which the carrier is other than gelatin, e. g., a resinous substance or cellulosic material which has no deteriorating effect on the light-sensitive materials. The dicarbocyanine dyes and heterocyclic bases can be employed in various concentrations depending upon the effects desired.

Ordinarily, the optimum or near optimum concentration of the dicarbocyanine dyes which we employ in practicing our invention is of the order of from 0.010 to 0.30 g. per mol. of silver halide in the emulsion.

The heterocyclic bases which we employ in our invention can advantageously be employed at a concentration of from about 0.05 to 1.0 g. per mol. of silver halide in the emulsion.

In general, the ratio of concentration of dicarbocyanine dye to heterocyclic base can vary rather widely in our combinations, e. g., from 1:5 to 1:100 (by weight) in many cases.

The methods of incorporating sensitizing dyes and heterocyclic bases in silver halide emulsions are well known to those skilled in the art. While the dicarbocyanine dyes and heterocyclic bases can be directly dispersed in the emulsions, it is convenient to add the same in the form of solutions in appropriate solvents. Methanol, ethanol, pyridine, and the like have proven satisfactory for many of the dyes of Formula I and bases of Formulas II, III and IV. Mixtures of solvents, e. g., pyridine diluted with methanol or acetone, can also be used. The dicarbocyanine dyes and heterocyclic bases are dispersed in the finished emulsions and should be uniformly distributed throughout the emulsions. The following procedure is satisfactory: Stock solutions of the dicarbocyanine dyes and heterocyclic bases are prepared by dissolving the same in appropriate solvents as described above. Then, to the flowable gelatino-silver-halide emulsion, the desired amounts of the stock solution of one of the dyes (or heterocyclic bases) are slowly added, while stirring the emulsion. Stirring is continued until the dye is thoroughly incorporated in the emulsion. Then the desired amount of the stock solution of the heterocyclic base (or dye, if heterocyclic base has been added first) is slowly added to the emulsion, while stirring. Stirring is continued until the second solution is thoroughly incorporated. The supersensitized emulsion can then be coated out on a suitable support, such as glass, cellulose derivative film, resin film, or paper, to a suitable thickness and allowed to dry. The details of such coating methods are well known to those skilled in the art. The foregoing procedures and proportions are to be regarded only as illustrative. Clearly, our invention is directed to any silver halide emulsion containing a combination of the aforesaid dicarbocyanine dyes and heterocyclic bases whereby a supersensitizing effect is obtained.

The following examples will serve to illustrate further the manner of practicing out invention.

In Table I below, to different portions of the same batch of photographic gelatino-silver-bromide emulsion were added (1) a dicarbocyanine dye, such as those represented by Formula I above, and (2) a combination of the dicarbocyanine dye and heterocyclic base. Then the emulsions were held at about 50-52° C. for a short time and coated on a support, chill set, and dried. After exposure through a Wratten No. 25 filter, i. e., a filter which transmits substantially no light of wavelength shorter than about 580 mu, in an Eastman Type Ib sensi-

tometer, the film strips were processed for 3 minutes in a developer having the following composition:

|   |                                | Grams |
|---|--------------------------------|-------|
|   | N-methyl-p-aminophenol sulfate | 2.0   |
| 5 | Hydroquinone                   | 8.0   |
|   | Sodium sulfite (desiccated)    | 90.0  |
|   | Sodium carbonate (monohydrate) | 52.5  |
|   | Potassium bromide              | 5.0   |
|   | Water to make 1 liter.         |       |

10 The speed (red), gamma and fog for each of the coatings was then measured. The results are recorded in Table I.

TABLE I

| Example | Sensitizing Dye and Base (g./mol.<br>AgX)                                                    | Red Light Exposure |       |     |
|---------|----------------------------------------------------------------------------------------------|--------------------|-------|-----|
|         |                                                                                              | 30/E<br>Speed      | Gamma | Fog |
| 20      |                                                                                              |                    |       |     |
| 1.      | {(a) 3,3'-diethoxythiadcarbocyanine iodide (.045).<br>(b) dye (a) (.045) plus base 1 (.30) . | 4.35               | 1.54  | .06 |
| 2.      | {(c) dye (a) (.045).<br>(d) dye (a) (.045) plus base 6 (.15) .                               | 10.6               | 2.48  | .06 |
| 3.      | {(e) dye (a) (.045) plus base 7 (.15) .                                                      | 3.85               | 1.21  | .06 |
| 4.      | {(f) dye (a) (.045) plus base 28 (.15) .                                                     | 7.55               | 1.80  | .06 |
| 5.      | {(g) dye (a) (.045) plus base 8 (.15) .                                                      | 8.85               | 2.16  | .06 |
| 6.      | {(h) dye (a) (.045) plus base 9 (.15) .                                                      | 29.5               | 3.18  | .06 |
| 7.      | {(i) dye (a) (.045) plus base 10 (.15) .                                                     | 10.4               | 2.40  | .06 |
| 8.      | {(j) dye (a) (.045) plus base 11 (.15) .                                                     | 15.4               | 2.70  | .06 |
| 9.      | {(k) dye (a) (.045) .                                                                        | 8.25               | 2.48  | .06 |
| 10.     | {(l) dye (a) (.045) plus base 12 (.15) .                                                     | 15.8               | 1.92  | .06 |
| 11.     | {(m) dye (a) (.045) plus base 13 (.15) .                                                     | 4.25               | 1.52  | .06 |
| 12.     | {(n) dye (a) (.045) plus base 14 (.15) .                                                     | 27.5               | 2.62  | .06 |
| 13.     | {(o) dye (a) (.045) .                                                                        | 11.4               | 2.64  | .06 |
| 14.     | {(p) dye (a) (.045) .                                                                        | 9.5                | 2.72  | .06 |
| 15.     | {(q) dye (a) (.045) plus base 2 (.15) .                                                      | 4.05               | 1.30  | .06 |
| 16.     | {(r) dye (a) (.045) plus base 3 (.15) .                                                      | 5.6                | 1.84  | .06 |
| 17.     | {(s) dye (a) (.045) plus base 4 (.15) .                                                      | 12.5               | 2.7   | .06 |
| 18.     | {(t) dye (a) (.045) plus base 5 (.15) .                                                      | 7.2                | 2.1   | .06 |
| 19.     | {(u) dye (a) (.045) .                                                                        | 7.9                | 2.32  | .06 |
| 20.     | {(v) dye (a) (.045) plus base 17 (.15) .                                                     | 5.8                | 2.0   | .06 |
| 21.     | {(w) 3,3'-di- $\beta$ -hydroxyethylthiadcarbocyanine bromide (.045) .                        | 7.2                | 2.0   | .06 |
| 22.     | {(x) dye (a) (.045) plus base 29 (.15) .                                                     | 6.40               | 1.90  | .05 |
| 23.     | {(y) dye (a) (.045) plus base 28 (.15) .                                                     | 13.7               | 2.40  | .06 |
| 24.     | {(z) 3,3'-diethylthiadcarbocyanine iodide (.045) .                                           | 19.0               | 2.70  | .06 |
| 25.     | {(a') dye (a') (.045) .                                                                      | 5.6                | 2.1   | .06 |
| 26.     | {(b') dye (a') (.045) plus base 21a (.15) .                                                  | 7.6                | 2.7   | .05 |
| 27.     | {(c') dye (a') (.045) plus base 18 (.15) .                                                   | 25.5               | 3.1   | .05 |
| 28.     | {(d') dye (a') (.045) plus base 16 (.15) .                                                   | 2.7                | 2.9   | .06 |
| 29.     | {(e') dye (a') (.045) with base 21a (.15) .                                                  | 6.0                | 2.4   | .05 |
| 30.     | {(f') dye (a') (.045) with base 16 (.15) .                                                   | 10.9               | 3.1   | .05 |
| 31.     | {(g') dye (a') (.045) plus base 16 (.15) .                                                   | 5.6                | 3.1   | .10 |
| 32.     | {(h') 3,3'-diethyl-4,5,4',5'-dibenzo-thiadcarbocyanine iodide (.045) .                       | 20.5               | 3.0   | .07 |
| 33.     | {(i') dye (a') (.045) plus base 16 (.15) .                                                   | 7.6                | 3.2   | .07 |
| 34.     | {(j') dye (a') (.045) plus base 16 (.15) .                                                   | 15.8               | 3.1   | .07 |
| 35.     | {(k') 1'-dimethyl-2,2'-dicarbocyanine bromide (.045) .                                       | 15.8               | 3.1   | .07 |
| 36.     | {(l') dye (a') (.045) plus base 16 (.15) .                                                   | 2.8                | 2.4   | .34 |
| 37.     | {(m') dye (a') (.045) plus base 16 (.15) .                                                   | 8.8                | 2.8   | .12 |
| 38.     | {(n') dye (a') (.045) plus base 30 (.15) .                                                   | 4.05               | 1.30  | .06 |
| 39.     | {(o') dye (a') (.045) plus base 31 (.15) .                                                   | 14.7               | 2.60  | .06 |
| 40.     | {(p') dye (a') (.045) .                                                                      | 15.4               | 3.1   | .06 |
| 41.     | {(q') dye (a') (.045) plus base 32 (.15) .                                                   | 4.15               | 1.80  | .08 |
| 42.     | {(r') dye (a') (.045) .                                                                      | 6.9                | 1.30  | .06 |
| 43.     | {(s') dye (a') (.045) plus base 22 (.15) .                                                   | 4.6                | 1.9   | .06 |
| 44.     | {(t') dye (a') (.045) plus base 19 (.15) .                                                   | 17.3               | 2.6   | .06 |
| 45.     | {(u') dye (a') (.045) plus base 20 (.15) .                                                   | 6.3                | 2.2   | .05 |
| 46.     | {(v') dye (a') (.045) .                                                                      | 9.3                | 3.0   | .06 |
| 47.     | {(w') dye (a') (.045) plus base 23 (.15) .                                                   | 4.0                | 2.3   | .06 |
| 48.     | {(x') dye (a') (.045) plus base 23 (.15) .                                                   | 7.0                | 2.2   | .05 |
| 49.     | {(y') dye (a') (.045) plus base 24 (.15) .                                                   | 7.4                | 2.4   | .06 |
| 50.     | {(z') dye (a') (.045) plus base 25 (.15) .                                                   | 14.4               | 3.1   | .06 |
| 51.     | {(a'') dye (a') (.045) plus base 26 (.15) .                                                  | 45.5               | 2.9   | .06 |
| 52.     | {(b'') dye (a') (.045) plus base 21 (.15) .                                                  | 9.9                | 2.4   | .06 |
| 53.     | {(c'') dye (a') (.045) plus base 15 (.15) .                                                  | 16.9               | 2.8   | .06 |
| 54.     | {(d'') dye (a') (.045) plus base 27 (.15) .                                                  | 10.4               | 2.3   | .06 |
| 55.     | {(e'') dye (a') (.045) .                                                                     | 2.0                | .50   | .05 |
| 56.     | {(f'') dye (a') (.045) plus base 18 (.32) .                                                  | 18.0               | 1.8   | .06 |

In the above table, the coatings of Examples 2, 3, 4, 5, 6, 7, and 8 were made from the same batch of emulsion, the coatings of Examples 9, 10, 11, and 12 were made from the same batch of emulsion, the coatings of Examples 13, 14, 15, and 16 were made from the same batch of emulsion, the coatings of Examples 18 and 19 were made from the same batch of emulsion, the coatings of Examples 20 and 21 were made from the same batch of emulsion, the coatings of Examples 22 and 23 were made from the same batch of emulsion, the coatings of Examples 27 and 28 were made from the same batch of emulsion, the coatings of Examples 30, 31, and 32 were

made from the same batch of emulsion, and the coatings of Examples 33 to 39 were made from the same batch of emulsion. No measurements of coatings containing only the heterocyclic bases of Formula II alone are given, since numerous coatings at the concentration used in the table have shown that these bases alone have little or no measurable sensitizing effect on the emulsions.

Our invention is primarily directed to the ordinarily employed gelatino-silver-halide developing-out emulsions, e. g., gelatino-silver-chloride, -chlorobromide, -chloroiodide, -chlorobromiodide, -bromide and -bromiodide developing-out emulsions. Emulsions which form the latent image mostly inside the silver halide grains, such as the emulsions set forth in U. S. Patent 2,456,956, dated December 21, 1948, can also be employed in practicing our invention.

The emulsions prepared in accordance with our invention can be coated in the usual manner on any suitable support, e. g., glass, cellulose nitrate film, cellulose acetate film, polyvinyl-acetal resin film, paper or metal.

Photographic silver halide emulsions, such as those listed above, containing the supersensitizing combinations of our invention can also contain such addenda as chemical sensitizers, e. g., sulfur sensitizers (e. g., allyl thiocarbamide, thiourea, allylisothiocyanate, cystine, etc.), various gold compounds (e. g., potassium chloroaurate, auric trichloride, etc.) (see U. S. Patents 2,540,085; 2,597,856 and 2,597,915), various palladium compounds, such as palladium chloride (U. S. 2,540,086), potassium chloropalladate (U. S. 2,598,079), etc., or mixtures of such sensitizers; anti-foggants, such as ammonium chloroplatinate (U. S. 2,566,245), ammonium chloroplatinite (U. S. 2,566,263), benzotriazole, nitrobenzimidazole, 5-nitroindazole, benzidine, mercaptans, etc. (see Mees—“The Theory of the Photographic Process,” Macmillan Pub., 1942, page 460), or mixtures thereof; hardeners, such as formaldehyde (U. S. 1,763,533), chrome alum (U. S. 1,763,533), glyoxal (U. S. 1,870,354), dibrom-acrolein (Br. 406,750), etc.; color couplers, such as those described in U. S. Patent 2,423,730, Spence and Carroll U. S. Patent 2,640,776, etc.; or mixtures of such addenda. Dispersing agents for color couplers, such as those set forth in U. S. Patents 2,322,027 and 2,304,940, can also be employed in the above-described emulsions.

Such silver halide emulsions can also contain thiazolidones or other ultraviolet absorbing compounds, such as those described in Sawdy U. S. Patent 2,739,888, issued March 27, 1956. While certain emulsion addenda, such as certain ultraviolet compounds, and certain color-forming compounds cause de-sensitization or un-sensitizing effects, it has been found that the new combinations of our invention largely overcome such effects. Typical color-forming compounds which can be so employed include those in U. S. Patent 2,322,027 and the following:

#### Coupler:

- (1) 1-hydroxy-2-[ $\delta$ -(2',4'-di-tert.amylphenoxy) - n-butyl]-naphthamide (U. S. Patent 2,474,293)
- (2) 1-hydroxy-4-phenylazo-4'-(p - tert. - butylphenoxy)-2-naphthaniide (U. S. Patent 2,521,908)
- (3) 2-(2,4-di-tert.-amylphenoxyacetamino)-4,6 - dichloro-5-methyl phenol (Graham U. S. Patent 2,725,291)
- (4) 2-( $\alpha$ -di-tert.amylphenoxy-n-butyrylamino) - 4,6 - dichloro-t-methyl phenol
- (5) 6-{ $\alpha$ -{4-[ $\alpha$ -(2,4 - di - tert.amylphenoxy)butyramido]-phenoxy}acetamido} - 2,4 - dichloro - 3-methyl phenol
- (6) 2-[3' - (2',4'' - diamylphenoxy) - acetamido]-benzamido-4-chloro-5-methyl phenol
- (7) 1-(2',4',6'-trichlorophenyl)-3 - [3'-(2'',4''-di-tert.amylphenoxyacetamido) - benzamido] - 5-pyrazolone (U. S. Patent 2,600,788)

5

10

- (8) 1-(2',4',6'-trichlorophenyl)-3-[3''-(2'',4'' - di-tert.amylphenoxyacetamido)-benzamido]-4 - (p-methoxyphenylazo)-5-pyrazolone
- (9) N-(4 - benzoylacetaminobenzenesulfonyl) - N-( $\gamma$ -phenylpropyl) - p - toluidine (U. S. Patent 2,298,443)
- (10)  $\alpha$ -o-methoxybenzoyl- $\alpha$ -chloro-4-[ $\alpha$  - (2,4 - di-tert.-amylphenoxy)-n - butyramido] - acetanilide (McCrossen, U. S. Patent 2,728,658)
- (11)  $\alpha$ -{3 - [ $\alpha$  - (2,4 - di - tert.amylphenoxy)acetamido]-benzoyl}-2-methoxyacetanilide
- (12) 3-benzoylacetamido-4-methoxy-2',4' - di - tert. - amylphenoxy acetanilide
- (13) 4-benzoylacetamido-3-methoxy-2',4' - di - tert. - amylphenoxy acetanilide

20

25

30

35

40

45

50

55

55

The following table and examples will serve to illustrate the beneficial effects of our new supersensitizing combinations when employed in a photographic emulsion containing a dispersion of a coupler or color-forming compound. In Table II, these effects are illustrated for an ordinary photographic gelatino-silver-bromiodide emulsion containing 3,3'-diethyloxathiadicarbocyanine iodide (50 mg./mol. AgX). To one portion of the sensitized emulsion was added a coupler dispersion containing coupler No. 5 of the above list, while no coupler dispersion was added to the second portion. To an aliquot of each of these portions of emulsion was added a heterocyclic base as identified in the following table. Each of the emulsions was then digested for a short time at 50° C., coated, chill set and exposed in an Eastman Type Ib sensitometer through a Wratten No. 25 filter as in the case of the coatings for Table I. The coatings containing the coupler dispersion were held at 40° C. for one-half hour before coating onto the film base and subsequent exposure. The exposed coatings were then developed for about 3 minutes in a developer having the composition indicated above with respect to Table I. After exposure and development of the coatings, the relative red speed, gamma, and fog for the coatings was measured. The results are given in Table II below.

TABLE II

| Example           | Base<br>(g./mol.<br>AgX) | Without Dispersion |       |     | With Dispersion |       |     |
|-------------------|--------------------------|--------------------|-------|-----|-----------------|-------|-----|
|                   |                          | Speed              | Gamma | Fog | Speed           | Gamma | Fog |
| 41 <sup>(a)</sup> | none                     | 100                | 3.7   | .04 | 21              | .46   | .12 |
|                   | 35 (4.0)                 | 535                | 5.1   | .04 | 180             | 3.0   | .07 |
| 42 <sup>(a)</sup> | none                     | 100                | 2.9   | .05 | 36              | 2.0   | .14 |
|                   | 36 (0.4)                 | 395                | 3.6   | .05 | 280             | 2.7   | .12 |

The bis compounds represented by Formula III above are to be distinguished from bis compounds containing a substituent on the nitrogen atom shown in Formula III, such as the following compounds:

(37)



(38)



75



Compounds 37-40 above can also be employed advantageously in combination with the dicarbocyanine dyes of our invention, such as dye (a) of Table I. Such compounds as 37-40 above have chemical properties distinct from the heterocyclic bases of our invention. It is to be further understood that in ascertaining the heterocyclic bases of our invention as set forth above, such heterocyclic bases contain not more than 2 nitrogen atoms in any heterocyclic ring, i. e., from 1 to 2 nitrogen atoms in any heterocyclic ring. As noted above,  $R_3$  of Formula IV can represent an alkylmercapto group, such groups including butylmercapto, hexylmercapto, octylmercapto, decylmercapto, dodecylmercapto, etc., (especially alkylmercapto groups containing from 4 to 12 carbon atoms).  $R_3$  of Formula IV can also represent an arylmercapto group as noted above, including phenylmercapto, tolylmercapto, etc., (especially an arylmercapto group containing from 4 to 7 carbon atoms). Particularly useful substituted imino groups ( $R_3$ ) of Formula IV include (heterocyclidene) ethylidene groups wherein the heterocyclic nucleus is the same or different type of heterocyclic nucleus represented by  $Z_3$ .

The accompanying drawing illustrates the supersensitizing effect obtained with three of our new combinations in gelatino-silver-bromiodide emulsions. Each figure of the drawing is a diagrammatic reproduction of two spectrograms. The sensitivity of the emulsion containing only the dicarbocyanine dye of Formula I is represented by the solid curve, while the sensitivity of the same emulsion containing both a dicarbocyanine dye of Formula I and a heterocyclic base, such as is represented by Formulas II, III or IV, is represented by the broken line. No curve representing the sensitivity of the heterocyclic base alone is shown, since numerous coatings at the concentrations shown in the table have indicated that these heterocyclic bases have little or no measurable sensitizing action of their own.

In Fig. 1, curve A represents the sensitivity of an ordinary gelatino-silver-bromiodide emulsion sensitized with 3,3'-diethylthiadicarbocyanine iodide, while curve B represents the sensitivity of the same emulsion sensitized with 3,3'-diethylthiadicarbocyanine iodide and 1,4-bis[2-(5-phenyloxazolyl)]benzene. Sensitometric measurements for these coatings are given in Example 21 of Table I.

In Fig. 2, curve C represents the sensitivity of an ordinary gelatino-silver-bromiodide emulsion sensitized with 3,3'-diethylthiadicarbocyanine iodide, while curve D represents the sensitivity of the same emulsion sensitized with 3,3'-diethylthiadicarbocyanine iodide and 1,2-bis(2-benzothiazolyl)ethylene. Sensitometric measurements for these coatings are given in Example 20 of Table I.

In Fig. 3, curve E represents the sensitivity of an ordinary gelatino-silver-bromiodide emulsion sensitized with 3,3'-diethyloxadicarbocyanine iodide, while curve F represents the sensitivity of the same emulsion sensitized with 3,3'-diethyloxadicarbocyanine iodide with 1,4-bis[2-(5-phenyloxazolyl)]benzene. Sensitometric measurements for these coatings are given in Example 25 of Table I.

Many of the heterocyclic bases represented by Formulas II, III and IV above have been previously described in the prior art. Listed below are references describing the method whereby a number of these compounds can be prepared, together with the melting point of these products in certain cases.

| Compound | Method Described in—                      | M. P. ° C.           |
|----------|-------------------------------------------|----------------------|
| 10       |                                           |                      |
| 2.       | Ber. 46, 97 and 13, 21                    | 133-5                |
| 3.       | do                                        | 75-6                 |
| 4.       | do                                        | 103-4                |
| 5.       | do                                        | 46-7                 |
| 6.       | Gazz. Chim. Ital., 62 (1932), 775         | 93-4                 |
| 7.       | do                                        | (B. P. 144-6/2 mm.). |
| 15       |                                           |                      |
| 9.       | J. Gen. Chem. U.S.S.R., 14 (1944), 865-80 | 213-4                |
| 10.      | Ber. 46, 97 and 13, 21                    |                      |
| 11.      | do                                        |                      |
| 12.      | J. Gen. Chem. U.S.S.R., 14 (1944), 865-80 | 190-4                |
| 13.      | Chem. Abs., 47 (1953), 2750               |                      |
| 14.      | Ber. 13, 21 and Ber. 46, 97               |                      |
| 15.      | Fr. Pat. 900,722                          |                      |
| 20       |                                           |                      |
| 17.      | Ber. 13, 21 and 46, 97                    |                      |
| 18.      | Fr. Pat. 900,722                          |                      |
| 19.      | U. S. 2,143,920                           |                      |
| 20.      | Ann. 14, 77                               |                      |
| 21a      | U. S. 2,483,392                           |                      |
| 26.      | Chem. Abs., 44 (1950), 6313               |                      |
| 27.      | Chem. Abs. 31, 1406                       |                      |
| 25       |                                           |                      |
| 31.      | Chem. Abs. 26, (1932), 1281               |                      |
| 32.      | J. A. C. S., 73, (1951), 1093             |                      |
| 33.      | U. S. 2,382,714                           |                      |
| 34.      | do                                        |                      |
| 35.      | Ann. 588, 10                              |                      |
| 38.      | U. S. 2,520,358                           |                      |
| 39.      | U. S. 2,739,964                           |                      |
| 40.      | Br. 461,688                               |                      |

The following examples describe the preparation of a number of these heterocyclic bases which can be employed in our invention.

35 Example A.—2-[4-(2-amino-5-methylphenylazo)phenyl]benzothiazole

A solution of 0.8 g. of sodium nitrite in 5 ml. of water was added dropwise to a cold (5° C.) suspension of 2.26 g. of 2-p-aminophenylbenzothiazole in 50 ml. of water containing 4 ml. of concentrated hydrochloric acid. The reaction mixture was allowed to stand in the cold for one hour, then diluted to 500 ml. with ice water and 0.5 g. of urea was added. The reaction mixture was filtered and the clear cold filtrate was added to 1.07 g. of p-toluidine dissolved in 5 ml. of pyridine. After standing for several hours the crystals were collected on a filter. The yield of product was 81% crude and 50% after two recrystallizations from benzene. The yellow crystals had M. P. 190-191° C. with decomposition.

50 Example B.—N,N'-bis(2-benzothiazolyl)oxamide

A mixture of 1.5 g. of 2-aminobenzothiazole and 1.46 g. of diethyl oxalate was heated under reflux for about two minutes. The solid product was removed from the flask and washed with methyl alcohol. After two recrystallizations from pyridine, the colorless crystals melted above 320° C.

60 Example C.—2-(2-benzothiazolylhydrazono)-methylbenzothiazole

A solution of 1.7 g. (1 mol.) of benzothiazole-2-carboxaldehyde and 1.7 g. (1 mol.) of 2-hydrazinobenzothiazole in 25 ml. of absolute ethyl alcohol was heated at the refluxing temperature for 30 minutes. After chilling, the product was collected on a filter and washed with ethyl alcohol. After two recrystallizations from a mixture of 30 percent pyridine and 70 percent ethyl alcohol, the yield was 37 percent, and the yellow crystals melted at 271-272° C. with decomposition.

70 Example D.—1,5-bis(2-benzothiazolylthio)pentane

A mixture of 8.35 g. (0.05 mol.) of mercaptobenzothiazole and 5.75 g. (0.025 mol.) of pentamethylene bromide was heated for two hours at 135° C. A homogeneous liquid first formed but soon solidified to a glassy

## 13

solid. The mixture was retained at 135° C. for two hours. The solid product was dissolved in methanol, decolorized with decolorizing carbon, filtered, and chilled. The solid that separated (4 g.) melted at 69° C. The higher melting solid is the salt which loses hydrogen bromide readily. A reaction carried out in methanol in the presence of sodium methoxide gave the same product.

Compound 16 can be prepared according to the method described in U. S. Patent 2,726,246, issued December 6, 1955.

Compound 21 was prepared in the manner shown in Example D above, by reacting together 2-mercaptopbenzimidazole and ethylene bromide.

Compound 24 was prepared as follows: 3.7 g. of 2-aminobenzothiazole was mixed with 2.1 ml. of diketene and allowed to stand. In about 10 minutes, a vigorous reaction took place. The mixture liquified and then turned to a solid. This solid was crystallized from alcohol to give a quantitative yield of product melting at 219° C.

Compound 36 was prepared as follows: 6.0 g. of the sodium salt of Compound 35 were dissolved in 100 ml. of water containing 5 g. of sodium carbonate. Phosgene was led into this solution at 50° C. with good stirring for a period of 1.5 hours. When the reaction mixture gave a negative diazo reaction, heating was discontinued and the desired product recovered from the reaction mixture by the addition of an equal volume of saturated salt solution. The yield of product was 4.3 g.

Compound 37, can be prepared by condensing 3-ethyl-2(3)-benzothiazolone hydrozone (Chem. Abs., 22, 1358) with terephthalic aldehyde.

What we claim as our invention and desire secured by Letters Patent of the United States is:

1. A photographic gelatino-silver-halide developing-out emulsion sensitized with a supersensitizing combination of at least one dicarbocyanine dye selected from those represented by the following general formula:



wherein R and R<sub>1</sub> each represents an alkyl group containing from 1 to 2 carbon atoms, n represents a positive integer of from 1 to 2, X represents an acid radical, Z represents the non-metallic atoms necessary to complete a heterocyclic nucleus selected from the group consisting of those of the benzothiazole series, those of the naphthothiazole series, those of the benzoselenazole series, those of the naphthoselenazole series, those of the benzoxazole series, those of the naphthoxazole series, those of the 2-quinoline series, those of the 4-quinoline series, and those of the benzimidazole series, and Z<sub>1</sub> represents the non-metallic atoms necessary to complete a heterocyclic nucleus selected from the group consisting of those of the benzoxazole series, those of the naphthoxazole series, those of the benzoselenazole series, those of the naphthoselenazole series, those of the benzothiazole series, those of the naphthothiazole series, and those of the 2-quinoline series, and at least one heterocyclic base selected from those represented by the following general formula:



wherein Z<sub>2</sub> represents the non-metallic atoms necessary to complete a heterocyclic nucleus selected from the group consisting of those of the thiazole series, those of the benzothiazole series, those of the naphthothiazole series, those of the oxazole series, those of the benzoxazole series, those of the naphthoxazole series, those of the selenazole series, those of the benzoselenazole series, those of the naphthoselenazole series, those of the benzimidazole series, and those of the 2-quinoline series, d

75

wherein R and R<sub>1</sub> each represents an alkyl group contain-

## 14

represents a positive integer of from 1 to 2, D represents a divalent organic radical selected from the group consisting of dithiaalkylene group containing from 1 to 5 carbon atoms, an alkylene group containing from 1 to 10 carbon atoms, an arylene group containing from 6 to 13 carbon atoms, a vinylene group, a thio group, and an oxydimethylene group.

2. A photographic gelatino-silver-halide developing-out emulsion sensitized with a supersensitizing combination of at least one dicarbocyanine dye selected from those represented by the following general formula:



wherein R and R<sub>1</sub> each represents an alkyl group containing from 1 to 2 carbon atoms, X represents an acid radical, and Z represents the non-metallic atoms necessary to complete a heterocyclic nucleus of the benzothiazole series, and at least one heterocyclic base selected from those represented by the following general formula:



25 wherein Z<sub>2</sub> represents the non-metallic atoms necessary to complete a heterocyclic nucleus selected from the group consisting of those of the thiazole series, those of the benzothiazole series, those of the naphthothiazole series, those of the oxazole series, those of the benzoxazole series, those of the naphthoxazole series, those of the selenazole series, those of the benzoselenazole series, those of the naphthoselenazole series, those of the benzimidazole series, and those of the 2-quinoline series, d

30 represents a positive integer of from 1 to 2, D represents a divalent organic radical selected from the group consisting of a dithiaalkylene group containing from 1 to 5 carbon atoms, an alkylene group containing from 1 to 10 carbon atoms, an arylene group containing from 6 to 13 carbon atoms, a vinylene group, a thio group, and an oxydimethylene group.

35 3. A photographic gelatino-silver-halide developing-out emulsion sensitized with a supersensitizing combination of at least one dicarbocyanine dye selected from those represented by the following general formula:



40 wherein R and R<sub>1</sub> each represents an alkyl group containing from 1 to 2 carbon atoms, X represents an acid radical, and Z represents the non-metallic atoms necessary to complete a heterocyclic nucleus of the benzothiazole series, and at least one heterocyclic base selected from those represented by the following general formula:



45 wherein Z<sub>2</sub> represents the non-metallic atoms necessary to complete a heterocyclic nucleus of the oxazole series and D represents an arylene group containing from 6 to 13 carbon atoms.

50 4. A photographic gelatino-silver-halide developing-out emulsion sensitized with a supersensitizing combination of 3,3'-diethylthiadicarbocyanine iodide and 1,4-bis(5-phenyl-2-oxazolyl)-benzene.

55 5. A photographic gelatino-silver-halide developing-out emulsion sensitized with a supersensitizing combination of at least one dicarbocyanine dye selected from those represented by the following general formula:



ing from 1 to 2 carbon atoms, X represents an acid radical, Z represents the non-metallic atoms necessary to complete a heterocyclic nucleus of the benzothiazole series, and Z<sub>1</sub> represents the non-metallic atoms necessary to complete a heterocyclic nucleus of the benzoxazole series, and at least one heterocyclic base selected from those represented by the following general formula:



5

wherein Z<sub>2</sub> represents the non-metallic atoms necessary to complete a heterocyclic nucleus selected from the group consisting of those of the thiazole series, those of the benzothiazole series, those of the naphthothiazole series, those of the oxazole series, those of the benzoxazole series, those of the naphthoxazole series, those of the selenazole series, those of the benzoselenazole series, those of the naphthoselenazole series, those of the benzimidazole series, and those of the 2-quinoline series, d represents a positive integer of from 1 to 2, D represents a divalent organic radical selected from the group consisting of a dithiaalkylene group containing from 1 to 5 carbon atoms, an alkylene group containing from 1 to 10 carbon atoms, an arylene group containing from 6 to 13 carbon atoms, a vinylene group, a thio group, and an oxydimethylene group.

6. A photographic gelatino-silver-halide developing-out emulsion sensitized with a supersensitizing combination of at least one dicarbocyanine dye selected from those represented by the following general formula:



wherein R and R<sub>1</sub> each represents an alkyl group containing from 1 to 2 carbon atoms, X represents an acid radical, Z represents the non-metallic atoms necessary to complete a heterocyclic nucleus of the benzothiazole series, and Z<sub>1</sub> represents the non-metallic atom necessary to complete a heterocyclic nucleus of the benzoxazole series, and at least one heterocyclic base selected from those represented by the following general formula:



wherein Z<sub>2</sub> represents the non-metallic atoms necessary to complete a heterocyclic nucleus of the benzothiazole series and D represents a bis(phenylene)methyl group.

7. A photographic gelatino-silver-halide developing-out emulsion sensitized with a supersensitizing combination of 3,3'-diethyloxathiadicarbocyanine iodide and bis-[4-(2-benzothiazolyl)-phenyl]methane.

8. A photographic gelatino-silver-halide developing-out emulsion sensitized with a supersensitizing combination of at least one dicarbocyanine dye selected from those represented by the following general formula:



wherein R and R<sub>1</sub> each represents an alkyl group containing from 1 to 2 carbon atoms, X represents an acid radical, and Z represents the non-metallic atoms necessary to complete a heterocyclic nucleus of the benzothiazole series, and at least one heterocyclic base selected from those represented by the following general formula:



10

wherein Z<sub>2</sub> represents the non-metallic atoms necessary to complete a heterocyclic nucleus selected from the group consisting of those of the thiazole series, those of the benzothiazole series, those of the naphthothiazole series, those of the oxazole series, those of the benzoxazole series, those of the naphthoxazole series, those of the selenazole series, those of the benzoselenazole series, those of the naphthoselenazole series, those of the benzimidazole series, and those of the 2-quinoline series, d represents a positive integer of from 1 to 2, D represents a divalent organic radical selected from the group consisting of a dithiaalkylene group containing from 1 to 5 carbon atoms, an alkylene group containing from 1 to 10 carbon atoms, an arylene group containing from 6 to 13 carbon atoms, a vinylene group, a thio group, and an oxydimethylene group.

15

9. A photographic gelatino-silver-halide developing-out emulsion sensitized with a supersensitizing combination of at least one dicarbocyanine dye selected from those represented by the following general formula:



30 35 wherein R and R<sub>1</sub> each represents an alkyl group containing from 1 to 2 carbon atoms, X represents an acid radical, and Z represents the non-metallic atoms necessary to complete a heterocyclic nucleus of the benzoselenazole series, and at least one heterocyclic base selected from those represented by the following general formula:



40 45 wherein Z<sub>2</sub> represents the non-metallic atoms necessary to complete a heterocyclic nucleus of the oxazole series and D represents an arylene group containing from 6 to 13 carbon atoms.

10. A photographic gelatino-silver-halide developing-out emulsion sensitized with a supersensitizing combination of 3,3'-diethylselenadicarbocyanine iodide and 1,4-bis(5-phenyl-2-oxazolyl)benzene.

#### References Cited in the file of this patent

#### UNITED STATES PATENTS

55 2,680,686 Van Dormael et al. ----- June 8, 1954